

Oct. 6, 1936.

F. WINKLER ET AL

2,056,914

THERMAL TREATMENT OF HYDROCARBONS

Filed March 18, 1933



INVENTORS  
FRITZ WINKLER  
HANS HAEUBER

BY *Hans Haub*  
ATTORNEYS

Patented Oct. 6, 1936

2,056,914

# UNITED STATES PATENT OFFICE

2,056,914

## THERMAL TREATMENT OF HYDROCARBONS

Fritz Winkler and Hans Haeuber, Ludwigshafen-on-the-Rhine, Germany, assignors to L. G. Farbenindustrie Aktiengesellschaft, Frankfort-on-the-Main, Germany

Application March 18, 1933, Serial No. 661,632  
In Germany March 22, 1932

2 Claims. (Cl. 196—133)

The present invention relates to the thermal treatment of hydrocarbons.

It has already been proposed to employ elements of the 4th group of the periodic system as catalysts or as coatings for the walls of the reaction vessels in the thermal treatment of hydrocarbons.

For this purpose, silicon in the free elementary form or in the form of alloys has proved especially valuable.

While, when employing carbon it is easy to deposit it in crystalline graphitic form from its gaseous compounds, and while moreover the metals of low melting point of the 4th group of the periodic system, such as tin or lead, may be readily applied to metallic substrata, it has only been possible hitherto to prepare with difficulty firmly adherent coatings, impermeable to gases, from the elements of high melting point of the 4th group of the periodic system, such as silicon or titanium, without the assistance of binding agents, especially those of ceramic nature, fluxes or the like.

We have now found that in the thermal treatment of hydrocarbon products in the solid, liquid or gaseous phase at any pressure in spaces confined by heat-resistant metals, as for example in tubes of ordinary iron or, for example, of iron alloys containing nickel, no trace of injurious deposition of carbon is obtained in continuous operation when the metallic surfaces which come into contact with the substances to be treated are provided wholly or in part with coatings of elements of the 4th group of the periodic system having a melting point between 1000° and 2000° C., which have been prepared by burning in the said elements in pulverulent form.

The burning temperature lies below the melting temperature of the element to be burned in and below the melting point of metal serving as the carrier material, but above about 950° C. Generally speaking with silicon or titanium it is between 1050° and 1150° C. and the period during which the elements remain in the glowing zone is from about 1 to 2 hours. If desired, the burning may be effected in a non-oxidizing, preferably reducing atmosphere, as for example in an atmosphere of nitrogen or hydrogen. In order to obtain a uniform surface it is preferable to free the metallic surface to be provided with a coating from the impurities, as for example metal oxides, adhering thereto. The material to be burned in is preferably employed in the form of finest powder in order to ensure that this material attaches most closely to the metallic walls. For example if it is desired to provide tubes with an internal protective layer, it has been found preferable in order to obtain a good application of the powder to fill the tubes with powder and to burn them in a vertical position. The dura-

tion of the burning or glowing depends on the external conditions, such as the kind of furnace employed, the thickness of the walls of the tubes or, for example when burning in silicon, on the outer surface of the tubes, on the thickness of the surrounding layer of powder and the like; in each case the said duration is preferably ascertained by preliminary experiment, for example by proving whether the tube coated with silicon is stable to mineral acids or like methods.

When employing ordinary iron tubes as the substrata, it is advantageous to make use of the known fact that silicon or titanium steels are especially stable to temperature and corrosion and to provide ordinary iron tubes, for example, with the protective layer both inside and outside, while when working with alloyed steels it is only necessary to apply the coating to the surfaces with which the hot substances to be treated come into contact.

By the employment of alloyed steels, as for example of V2A-steel consisting of about 72 per cent of iron, 7 per cent of nickel, and 20 per cent of chromium, especially firmly adherent coatings are obtained.

As processes for which the apparatus so produced may be used may be mentioned, *inter alia*, dry distillation of solid fuels, distillation of liquid hydrocarbons, cracking or dehydrogenation of hydrocarbons in the liquid or vapor phase or polymerization of gaseous or liquid hydrocarbons under the influence of high temperature at atmospheric or increased pressure, as for example the conversion of paraffinic or olefinic hydrocarbons into aromatic hydrocarbons if desired in the presence of indifferent gases or gases taking part in the reaction. For these treatments temperatures between 300° and 1100° C. depending upon the particular conversion come into question.

The invention will be further explained with reference to the accompanying drawing showing a longitudinal section of a tube in which the said conversions of hydrocarbons may be carried out. It is to be understood, however, that the invention is not restricted to the particular arrangement shown in the drawing.

In this drawing *a* denotes an iron tube which is internally coated with a layer *b* of silicon burnt thereinto as a powder. The tube is heated from outside by any desired heating means (not shown) such as hot gases or by electric heat supply. The gas to be converted is introduced at *c*; the gas having undergone conversion leaves the tube at *d*.

The following examples will further illustrate the nature of this invention but the invention is not restricted to these examples.

### Example 1

A tube, about 5 meters long, of chromium nickel steel having an internal diameter of about 15

millimeters and an external diameter of about 22 millimeters is filled with fine silicon powder and kept for about an hour at from about 1050° to 1100° C. in a vertical furnace. The tube is then allowed to cool and the silicon powder which has not been burnt on is removed, the tube then being ready for use.

The tube is arranged vertically in one of the usual cracking apparatus for the cracking of petroleum of high boiling point in the vapor phase and is heated externally by fire gases so that the temperature in the middle of the tube is 780° C., at the lower end 750° C. and at the upper end 700° C. From about 5 to 6 kilograms of the middle fraction, boiling above 200° C., of a German petroleum are led in the vapor phase per hour through the tube with an addition of about 1 cubic meter of the final gas obtained in the cracking process which has been freed from condensable cracking products.

By a single passage through the tube about 18 to 20 per cent by weight of a benzine boiling below 200° C., about 65 per cent of residual oil which is added to the initial material, about 3 to 5 per cent of non-vaporizable heating oil and from 10 to 15 per cent of gaseous constituents are obtained.

The final gas has approximately the following composition, the percentages being by volume:

|                                | Per cent      |
|--------------------------------|---------------|
| H <sub>2</sub>                 | 12.5          |
| C <sub>2</sub> H <sub>4</sub>  | 21.5          |
| C <sub>3</sub> H <sub>8</sub>  | 18.5          |
| C <sub>4</sub> H <sub>8</sub>  | 7.5           |
| CH <sub>4</sub>                | 24.0          |
|                                | Per cent      |
| C <sub>2</sub> H <sub>6</sub>  | 5.0           |
| C <sub>3</sub> H <sub>8</sub>  | 7.0           |
| C <sub>4</sub> H <sub>10</sub> | 4.0           |
|                                | 16.0 per cent |

After using the tube continuously for more than two months no injurious deposition of carbon can be detected.

The tube treated with silicon is equally suitable for the dehydrogenation of saturated benzines for the production of anti-knock motor fuels.

#### Example 2

A gas having the composition:

|                                | Per cent by volume |
|--------------------------------|--------------------|
| CH <sub>4</sub>                | 8.05               |
| C <sub>2</sub> H <sub>6</sub>  | 14.20              |
| C <sub>3</sub> H <sub>8</sub>  | 51.85              |
| C <sub>4</sub> H <sub>10</sub> | 11.90              |
| C <sub>2</sub> H <sub>4</sub>  | 4.45               |
| C <sub>3</sub> H <sub>6</sub>  | 4.80               |
| C <sub>4</sub> H <sub>8</sub>  | 0.95               |
| H <sub>2</sub>                 | 2.20               |
| N <sub>2</sub>                 | 1.40               |
| O <sub>2</sub>                 | 0.05               |
| CO                             | 0.15               |

is led at the rate of 12 liters per hour downwards through a chromium iron tube 1 meter in length and 15 millimeters in internal diameter which has been treated with silicon internally as described in Example 1 and which is heated in an electric furnace so that the upper about 60 centimeters thereof are at 650° C. while the about 20 centimeters therebelow are at about 800° C.

From each liter of the initial gas, 1.58 liters of a gas are obtained having the following composition, the percentages being by volume:

|                                | Per cent |
|--------------------------------|----------|
| CH <sub>4</sub>                | 30.90    |
| C <sub>2</sub> H <sub>6</sub>  | 8.15     |
| C <sub>3</sub> H <sub>8</sub>  | 2.15     |
| C <sub>4</sub> H <sub>10</sub> | 0.15     |
| C <sub>2</sub> H <sub>4</sub>  | 30.70    |
| C <sub>3</sub> H <sub>6</sub>  | 5.00     |
| C <sub>4</sub> H <sub>8</sub>  | 0.50     |
| H <sub>2</sub>                 | 21.40    |
| N <sub>2</sub>                 | 0.86     |
| O <sub>2</sub>                 | 0.03     |
| CO                             | 0.16     |

Furthermore 15.6 per cent by weight of the initial gas are converted into liquid products of which about 85 per cent consist of products boiling up to 200° C. and mainly composed of aromatic hydrocarbons.

In this case also no inconvenience is caused by the deposition of carbon even after operation for long periods of time.

If titanium be burnt in instead of silicon, the same results are obtained. Titanium is burnt in also in pulverulent form in a non-oxidizing atmosphere and preferably at a temperature between 1050° and 1150° C.

What we claim is:

1. A process for heat-treating a hydrocarbon product at a temperature between 300° and 1100° C., which comprises confining said product at the said temperature in a space enveloped by a heat-resistant metal which is internally coated with a layer substantially consisting of an element of the 4th group of the periodic system having a melting point between 1000° and 2000° C. burnt in the said metal in pulverulent form.

2. A process for heat-treating a hydrocarbon product at a temperature between 300° and 1100° C., which comprises confining said product at the said temperature in a space enveloped by a metal selected from the group consisting of iron and iron alloys which is internally coated with a layer substantially consisting of an element selected from the group consisting of silicon and titanium burnt in the said metal in pulverulent form.

FRITZ WINKLER.  
HANS HAEUBER.